

Feb. 13, 1940.

G. A. RICHTER

2,190,193

CHEMICAL WOOD-PULPING PROCESS

Filed Jan. 31, 1936



Inventor  
George A. Richter  
By Knight, Brown, DeWitt & May  
Attest

## UNITED STATES PATENT OFFICE

2,190,193

## CHEMICAL WOOD-PULPING PROCESS

George A. Richter, Berlin, N. H., assignor to  
 Brown Company, Berlin, N. H., a corporation  
 of Maine

Application January 31, 1936, Serial No. 61,678

6 Claims. (Cl. 92—13)

This invention relates to various chemical wood-pulping processes and more particularly to those wherein a cooking liquor containing caustic soda is employed for pulping chipped wood. Its 5 objective is the pulping of chipped wood under conditions such that the resulting pulp excels that produced by the usual processes in tear resistance, bleachability, and other respects.

In producing chemical wood pulps it is sometimes the practice to use cooking liquors containing caustic soda as an essential or principal fiber-liberating chemical. Thus, so-called kraft or sulphate pulp is produced by cooking the raw chipped wood in a liquor wherein caustic soda and sodium sulphide serve as the essential fiber-liberating chemicals. Again, so-called soda pulp derives its name from the caustic soda-containing cooking liquor in which it is produced, namely, a liquor containing practically only caustic soda as the 10 active pulping chemical. And there are modifications of these processes based on the use of liquors containing caustic soda and sodium sulphite or containing caustic soda, sodium sulphite, and sodium sulphide as the pulping agents. All 15 of these processes, however, are performed similarly in the respects that the cooking is effected with an amount of liquor only moderately in excess of that required to cover the chips and containing fiber-liberating chemical only moderately 20 in excess of that consumed or spent by reaction with the ligneous or encrusting components of the wood.

In accordance with the present invention, wood pulp is produced by cooking appropriately chipped wood in a sodium base alkaline liquor of the character hereinbefore described in volume more than twice that requisite for covering the wood and containing fiber-liberating chemical more than 25 twice that requisite for complete pulping or fiber liberating action, for I have found that wood pulp thus produced is of notably better quality than the pulps heretofore produced. It is thus seen that the process hereof involves cooking 30 wood in a liquor whose active sodium content based on wood is much greater than that of the liquors heretofore used but whose active sodium concentration is not necessarily in excess of that of the liquors heretofore used. Indeed, in some 35 instances, the cooking liquors of the present invention may be no more concentrated or even less concentrated in active sodium constituent than the liquors heretofore used even though they are associated in such volume with the wood as 40 to contain more than twice the amount of active

sodium constituent necessary to accomplish complete pulping or fiber liberation.

While it is possible to embody the principles of the present invention in various specific pulping processes performed with sodium base alkaline 5 liquors, I shall now illustrate how these principles may be applied advantageously in the pulping of wood by a so-called kraft cooking liquor containing both caustic soda and sodium sulphide as the fiber-liberating chemicals. Spruce chips, such as 10 are ordinarily prepared for kraft cooking, are put into a digester together with a sufficient volume of kraft cooking liquor containing 2 pounds of Na<sub>2</sub>O equivalent per cubic foot to provide a digester charge containing 0.4 pound of Na<sub>2</sub>O 15 equivalent per pound of bone dry wood. The liquor may be one whose sodium base exists essentially in the form of caustic soda and sodium sulphide, about 30 to 50% of its Na<sub>2</sub>O content, for instance, being in the form of sulphide. The 20 digester charge so made up, which includes a volume of liquor more than twice that necessary to cover the wood chips, may be cooked for about 4 hours at 335° F., at the end of which time the 25 chips are fully pulped and the digester contents 25 may be discharged into a blow tank wherein the liquor may be drained or otherwise separated from the pulp. The resulting pulp upon being washed has a so-called cooking stain value of about 115, which value is distinctly higher than 30 that of the ordinary commercial kraft pulp and indicates that the pulp is of distinctly lower ligneous content and may be bleached more readily and with lower bleach consumption than the ordinary commercial kraft pulp. When the pulp 35 is beaten to a predetermined degree and formed into test sheets of paper, it exhibits a tear resistance of at least about 300 as compared with a tear resistance of only about 250 in the case of the usual kraft pulp similarly tested. It might be observed that the foregoing comparison is based on 40 pulps derived from a particular kind of wood, namely, a Northern spruce which was reduced to a particular chip size preparatory to pulping. Although other woods, such as Southern pine, Western 45 fir, white birch and other hardwoods, etc., might yield pulps of different tear resistance values, such other woods when pulped by the process hereof yield in all cases pulps of decidedly better tear resistance, bleachability, and 50 other qualities than the pulps produced from the same woods by cooking as in the usual kraft process.

The foregoing improved results attained by the practice of the present invention are at- 55

tributable to the large excess of both cooking liquor and fiber-liberating chemical employed in the pulping of the wood. Thus, these results cannot be approached even when, as is true in the usual kraft process, the liquor contains a greater concentration of active sodium constituent, that is, is stronger, but is used in volume, relative to wood, much less than that used in the process hereof. For instance, even when a kraft liquor 5 contains as much as 3 pounds of Na<sub>2</sub>O equivalent per cubic foot of liquor, it yields wood pulp distinctly inferior to that produced hereby when it is associated or used with raw wood in such limited volume that the Na<sub>2</sub>O equivalent amounts 10 to, say, 0.2 pound per pound of wood, as may be true in the usual kraft process. On the other hand, when only the ratio of fiber-liberating chemical to wood is increased, the improved pulp product hereof is not realized. Thus, when pulping 15 of wood is accomplished in the usual volume of kraft cooking liquor, even though the liquor may be so concentrated as to contain 0.4 pound of Na<sub>2</sub>O equivalent per pound of dry wood, it does not yield the product hereof. On the contrary, 20 the resulting pulp generally has a tear resistance 25 even lower than that of the usual kraft pulp.

In the case of kraft liquors, a marked improvement is effected in the quality of the pulp when cooking of the wood takes place in a liquor whose 30 active Na<sub>2</sub>O content ranges from about 2 to 3 pounds per cubic foot and whose volume relative to wood is such that at least about 0.3 to 0.6 pound of active Na<sub>2</sub>O equivalent is present per pound of dry wood. These same active Na<sub>2</sub>O 35 values may be advantageously maintained in so-called soda liquor, that is, liquor wherein essentially all of the active sodium constituent is present as caustic soda, or in liquor wherein, besides caustic soda, part of the active sodium constituent exists as sodium sulphite or as sodium sulphite and sodium sulphide.

In the particular example hereinbefore described, wood chips of the usual size were cooked or pulped, that is, chips of about  $\frac{3}{4}$  to 1" length, 45 about  $\frac{3}{8}$  to  $\frac{1}{2}$ " width, and about  $\frac{1}{8}$  to  $\frac{1}{4}$ " thickness. However, it is possible to depart widely from such particular chip dimensions or size while pursuing the practice of the present invention. For instance, it is possible to chip 50 wood into much larger units or to comminute wood into fragments approximating sawdust and to pulp these various reduced forms of wood by the process hereof. When the objective hereof is a finished pulp possessed of high average fiber 55 length and good tear resistance as well as easy bleachability, it is preferable to use wood chips of the usual size or even larger, but, in those instances when the objective is a uniformly cooked pulp of easy bleachability, smaller than normal 60 wood units or fragments may advantageously be the form of cellulose subjected to the pulping operation. It is to be understood, therefore, that the expression "chipped wood" as used in the appended claims is meant to be inclusive of wood 65 chips or fragments of various sizes that may be pulped by the process hereof.

In practicing the process of the present invention, it is unnecessary to provide digesters of such size as to hold all the pulping liquor to act 70 upon the wood chips being pulped. Thus, it is possible to provide a tank or reservoir outside of the digesters for the purpose of holding the liquor in excess of that normally used and to cause such excess liquor while at the desired cooking temperature to circulate through the digesters 75

as cooking of the chips is taking place. I have shown diagrammatically in the accompanying drawing a system or arrangement of instrumentalities such as may be adopted in the practice of the present invention.

The numerals 10 represent a battery of digesters in which chipped wood may be cooked or pulped under the conditions hereinbefore described. After the pulping operation, the digester contents may be delivered into a series of 10 blow tanks 11, wherein the liquor may be separated, as by draining, from the pulp. The pulp may be sluiced from the blow tanks 11 to a suitable washer, for instance, to a countercurrent washer that dilutes the residual liquor washed 15 from the pulp to a minimum degree so that the valuable sodium constituent may be economically recovered from the liquor for reuse.

The liquor drained or otherwise separated from the pulp in the tanks 11 is rich in unconsumed or active pulping chemical and may hence be reused in the pulping of raw wood. Thus, whereas in the usual kraft process, the black or spent liquor contains largely spent alkali or Na<sub>2</sub>O equivalent, the sodium content of the used liquor 20 of the present invention is present largely as active or residual alkali. Such used liquor may be passed to a preheating tank 12 wherein it may be commingled with fresh alkali or so-called white liquor from a supply tank 13 in amount 25 sufficient to increase its active alkali content to that desired for the cooking of fresh wood. After the used liquor has been brought to the desired active alkalinity, it may be heated under pressure to the temperature, say, 335° F., to be maintained during cooking in the digesters 10, as by circulation from the closed tank 12 through a heater 14 back to such tank.

The liquor preheated to the desired temperature in the closed tank 12 may be passed to a 40 closed accumulator tank 15 having a vent line 16 communicating with the tank 12 so that air or steam to be displaced in the accumulator tank may be released into the closed tank 12. After the preheated liquor has been exhausted into 45 the accumulator tank 15, the valves in the pipelines connecting this tank with the preheating tank 12 may be closed and the air or steam in the preheating tank 12 may be released preparatory to running thereinto other used liquor to be 50 preheated. As soon as there is accumulation of the desired amount of preheated liquor in the tank 15, the liquor may be pumped therefrom into the digesters through their bottom ends so as to submerge or cover their charges of raw 55 chipped wood. The cooking of the chipped wood in the digesters takes place as liquor is withdrawn from the digesters at their upper ends and is passed to the accumulator tank 15 which may be provided with steam-heating coils or 60 other suitable heating means adapted to keep the liquor at the desired cooking temperature, for instance, 335° F. As cooking of the chipped wood in the digesters proceeds, liquor is constantly pumped into the lower end portions of 65 the digesters, and circulated back to the tank 15 which contains therein liquor in sufficient volume to produce the improved pulping action on the wood chips desired herein. In other words, the total volume of liquor in the system, that is, 70 the volume of liquor in the digesters and in the tank 15, is more than twice that necessary for covering the chips in all the digesters. Of course, the withdrawal of liquor at the top of digesters is effected at such a rate that the 75

chipped wood charge in each of the digesters is completely submerged by liquor at substantially uniform cooking temperature. It will be appreciated that no attempt has been made to illustrate the true relative proportions of the various instrumentalities in the drawing and that the drawing is to be regarded as being in the nature of a flow-sheet.

The particular pulping system hereinbefore described does away with the need for increasing digester capacity beyond that of usual digesters, since heating of practically all the excess liquor necessary for the purpose of the present invention may be done outside of the digesters while it is out of contact with the wood chips. It thus becomes possible to practice the present invention without building excessively large digesters of such strength or structural design as to be capable of withstanding the weight of both the chipped wood and all of the liquor participating in the pulping reaction. In other words, the large volume of excess liquor outside of the digesters is constantly maintained in circulatory contact with the wood being cooked in the digesters and thus conduces to substantially the same results as if all the liquor were present with the chipped wood in the digesters.

When cooking of wood is carried out with soda liquor or liquors containing caustic soda and sodium sulphite or caustic soda sodium sulphite and sodium sulphide, the very same system as that herein described and illustrated may be employed. In all such cases, the liquor should contain more than twice the amount of fiber-liberating chemical necessary to ensure complete pulping of the wood, but such chemical, rather than being present in the usual volume of liquor, is dissolved in a volume of liquor more than twice that necessary for covering the chips. It might be observed that the improved results of the present invention may be attributable to the fact that the concentration of active fiber-liberating chemical in the liquor does not undergo marked change during the cooking operation; and it is for this reason that the used liquor, that is, the liquor separated from the completely pulped chips, contains fiber-liberating chemical largely in active condition. Apparently, in the ordinary cooking processes the fiber is evidently injured toward the end stages of the cooking or pulping operation by reason of the fact that, as the concentration of unconsumed caustic soda and/or other fiber-liberating chemical is markedly reduced, the liquor tends to hydrolyze the fiber. On the other hand, in the cooking operation hereof, there is comparatively much smaller change in the concentration of the caustic soda and/or other fiber-liberating chemical as the cooking operation proceeds so that cooking or fiber-liberating action at the end stage of the cooking operation is about as intensive as at the early stage of the cooking operation and a more uniformly cooked pulp is realized in a given period of time; and, since the cooking liquor at the end of the cooking operation is quite rich in unconsumed caustic soda or other fiber-liberating chemical, there is less injury done to the fiber at the end-stages of cooking by reason of fiber-hydrolysis.

The process of the present invention is applicable to various kinds of woods, such as spruce, fir, pine, birch, maple, etc. In other words, softwoods and hardwoods of all sorts may be pulped as herein described.

I claim:

1. A process of pulping chipped wood in an alkaline sodium base cooking liquor containing caustic soda as an essential fiber-liberating chemical, which comprises cooking the chipped wood in a plurality of digesters each of which contains a volume of such liquor not much more than that necessary to cover said wood, said liquor having an active sodium constituent concentration, including caustic soda, from substantially the very beginning of the cooking operation amounting to about two to three pounds of  $\text{Na}_2\text{O}$  equivalent per cubic foot of liquor; and, during the cooking operation, maintaining circulatory communication between the liquor in said digesters and a sufficiently large reservoir of similar liquor outside of said digesters to cause a volume of liquor more than twice that requisite for covering the wood and corresponding to at least 0.3 to 0.6 pound of active  $\text{Na}_2\text{O}$  equivalent per pound of dry wood to participate in the cooking operation.

2. A process of pulping chipped wood in a cooking liquor containing caustic soda and sodium sulphide as its essential fiber-liberating chemicals, which comprises cooking the chipped wood in a plurality of digesters each of which contains a volume of such liquor not much more than that necessary to cover said wood, said liquor containing caustic soda and sodium sulphide in concentration, calculated as  $\text{Na}_2\text{O}$  equivalent, from substantially the very beginning of the cooking operation amounting to about two to three pounds per cubic foot of liquor; and, during the cooking operation, maintaining circulatory communication between the liquor in said digesters and a sufficiently large reservoir of similar liquor outside of said digesters to cause a volume of liquor more than twice that requisite for covering the wood and corresponding to 0.3 to 0.6 pound of  $\text{Na}_2\text{O}$  equivalent per pound of dry wood to participate in the cooking operation.

3. A process of pulping chipped wood in an alkaline sodium base cooking liquor containing caustic soda as an essential fiber-liberating chemical, which comprises cooking the chipped wood in a digester which contains a volume of such liquor not much more than that necessary to cover said wood; and maintaining during the cooking operation circulatory communication between the liquor in said digester and a sufficiently large reservoir of similar liquor outside of said digester to cause a volume of liquor more than twice that requisite for covering said wood to participate in the cooking operation, the total volume of liquor participating in the cooking operation containing far more than sufficient active fiber-liberating chemical to pulp said wood completely.

4. A process of pulping chipped wood in an alkaline sodium base cooking liquor containing caustic soda as an essential fiber-liberating chemical, which comprises cooking the chipped wood in a digester which contains a volume of such liquor not much more than that necessary to cover said wood; maintaining during the cooking operation circulatory communication between the liquor in said digester and a sufficiently large reservoir of similar liquor outside of said digester to cause a volume of liquor more than twice that requisite for covering said wood to participate in the cooking operation, the total volume of liquor participating in the cooking operation

- containing far more than sufficient active fiber-liberating chemical to pulp said wood completely; and heating the liquor while part of said reservoir outside of the digester substantially to the temperature of cooking in said digester.
5. A process of pulping chipped wood in an alkaline sodium base cooking liquor containing caustic soda as an essential fiber-liberating chemical, which comprises cooking the chipped wood in a digester which contains a volume of such liquor not much more than that necessary to cover said wood, said liquor having an active sodium constituent concentration, including caustic soda, amounting to about 2 to 3 pounds of  $\text{Na}_2\text{O}$  equivalent per cubic foot of liquor; maintaining during the cooking operation circulatory communication between the liquor in said digester and a sufficiently large reservoir of similar liquor outside of said digester to cause a volume of liquor more than twice that requisite for covering the wood and corresponding to at least 0.3 to 0.6 pound of active  $\text{Na}_2\text{O}$  equivalent per pound of dry wood to participate in the cooking operation; and heating the liquor while part of said reservoir
- 10
- 15

outside of the digester substantially to the temperature of cooking in said digester.

6. A process of pulping chipped wood in a cooking liquor containing caustic soda and sodium sulphite as its essential fiber-liberating chemicals, which comprises cooking the chipped wood in a plurality of digesters each of which contains a volume of such liquor not much more than that necessary to cover said wood, said liquor containing caustic soda and sodium sulphite in concentration, calculated as  $\text{Na}_2\text{O}$  equivalent, amounting to about 2 to 3 pounds per cubic foot of liquor; maintaining during the cooking operation circulatory communication between the liquor in said digesters and a sufficiently large reservoir 10 of similar liquor outside of said digesters to cause a volume of liquor more than twice that requisite for covering the wood and corresponding to 0.3 to 0.6 pound of  $\text{Na}_2\text{O}$  equivalent per pound of dry wood to participate in the cooking operation; and heating the liquor while part of said reservoir outside of the digesters substantially to the temperature of cooking in said digesters.

GEORGE A. RICHTER.